

United States Patent [19]  
Cooney

[11] 3,898,166  
[45] Aug. 5, 1975

[54] ORGANIC ANTISTATIC COMPOSITION

[75] Inventor: William J. Cooney, Hixson, Hamilton, Tenn.

[73] Assignee: GAF Corporation, New York, N.Y.

[22] Filed: Jan. 16, 1973

[21] Appl. No.: 324,141

[52] U.S. Cl. .... 252/8.75; 252/8.8; 252/545; 117/139.5 CQ; 117/139.5 F; 117/139.5 C

[51] Int. Cl. .... D06m 13/38

[58] Field of Search ..... 252/8.6, 8.75, 8.8, 545; 117/139.5 CQ, 139.5 F, 139.5 C

[56] References Cited

UNITED STATES PATENTS

|           |        |                |           |
|-----------|--------|----------------|-----------|
| 3,652,419 | 3/1972 | Karg .....     | 252/8.6 X |
| 3,658,573 | 4/1972 | Guestaux ..... | 252/8.6 X |

Primary Examiner—Stephen J. Lechert, Jr.  
Attorney, Agent, or Firm—Walter C. Kehm; James N. Blauvelt

[57] ABSTRACT

An antistatic composition particularly adapted for use on textiles, floor coverings, and related materials, comprising an aqueous liquid fluid medium, having a pH within the range of about 7 to 13 and containing as active ingredient an organic antistatic textile agent and from about 1 to 0.5 parts by weight of a humectant. The humectant may be either a nonionic humectant (such as glycerine) or an ionic humectant (including strong electrolytes such as calcium chloride). When the humectant is nonionic, there must also be present at least 0.01 part by weight of a strong electrolyte, i.e., the salt of a strong base and a strong acid.

16 Claims, 1 Drawing Figure



## ORGANIC ANTISTATIC COMPOSITION

## BACKGROUND OF THE INVENTION

This invention relates to an antistatic composition adapted for use on textiles, floor coverings and related materials. More specifically this invention relates to an antistatic composition particularly adapted for use on pile fabrics, especially carpeting and upholstery fabrics normally backed with polymeric coatings and on vinyl and asbestos sheet and tile flooring, polyurethane and polyolefin flooring and on linoleum petroleum composition flooring products and the like. This invention is also concerned with a process for the preparation of an antistatic composition, and a process for treating the above with same in order to reduce electrostatic charge build-up in textiles.

The phenomena whereby charges of static electricity are built up in textiles is an acute problem in textile forming and treating processes, and in the normal use of upholstery and carpeting fabrics. The same situation applies to the aforementioned floor coverings. Static charges are transferred to the individuals who are in contact with the wear layer of the textiles or floor coverings, who then may receive an unpleasant "shock" when the charge passes from the individual to the ground.

When two or more dielectric materials are rubbed together an electrostatic charge is generated. Due to the dielectric nature of the materials in question, the static charges are not dispersed. This charge build-up is particularly acute in an environment of low humidity. The conditions for generation of electrostatic charges are met when clothing of individuals is rubbed against upholstery fabrics or their shoes rub, or scuff against flooring, the conditions being particularly favorable for generation of charges of static electricity under the relatively low humidity conditions that are frequently present indoors during the winter months.

When a charge of static electricity has been built up in an individual he can be subjected to the discomfort of a slight "shock" or "spark," particularly when he touches a metallic object to ground himself. If the generated charges of electricity can be dispersed throughout the dielectrical material, textile and/or flooring, they will not build up in persons in contact therewith. The antistatic compositions of this invention allow charges of the subject type to be evenly dispersed throughout textile and textile-type materials, and said floor coverings.

As used in accordance with this invention the term "antistatic" pertains to reducing or eliminating the property or ability to generate, induce or accumulate electrostatic charges.

There are many prior art chemicals and compositions which can minimize this problem, for example, the composition as disclosed in U.S. Pat. Nos. 2,717,842, Vitalis; 2,809,159, Wells; 3,101,323, Merlo et al; and 3,519,561 Kelly et al. These prior art compositions have many defects and it can generally be said that they are not well suited for use on varying carpet structures. Some of the problems attendant with the use of these prior art antistatic compositions adversely affect the ability of textile surfaces to be dyed or otherwise decorated. Likewise, the prior art compositions often affect adversely the hand qualities of the textile. In many cases in order to be effective the prior art compositions must be applied to the fabric or carpet face. While this

is permissive for some applications, in most cases it tends to produce an unsightly surface and said coated areas tend to attract dirt, and in addition, the antistatic composition is more likely to be removed during normal use and cleaning of the textile or flooring. The composition of U.S. Pat. No. 3,519,561 while similar to the instant invention, differs in that the former tends to migrate to the surface of the textile structure when the latter is shampooed or merely wetted. Additionally, the latter referred to composition, exhibits a tendency to have a marked corrosive nature upon the equipment from which same is applied. This property is probably attributable to the low pH of the prior art composition and accordingly the use of these prior art antistatic coatings on carpets and upholstery is severely restricted.

## SUMMARY OF THE INVENTION

An object of this invention is the preparation of an improved antistatic composition.

Another object of this invention is the preparation of an antistatic composition which can be used in such a way that it does not attract dirt, is not worn off in normal use nor does same migrate to the surface of the textile structure when the latter is washed.

Likewise an object of this invention is the preparation of an antistatic composition which does not affect adversely the hand properties of the treated textile.

Still another object of the invention is the preparation of an antistatic composition which is compatible with the latex binders that are used as carpet backing and adhesives and is non-corrosive to the machinery from which same is applied to the textile structure.

Still other objects of this invention include the process for the preparation of the antistatic composition of this invention, the process for coating fabric therewith, a process for rendering textiles antistatic and a process for the reduction of static electricity charge build-up in humans in contact with flooring.

The antistatic material is effective without being in contact with the backing and the ends of the fibers of textiles or flooring wear layer. The amount of material applied as such antistatic coating should be normally from .01 to 20 ounces per square yard and preferably from 2.0 to 10.0 ounces per square yard of the antistatic coating as applied.

The antistatic coating composition employed for the antistatic coating herein comprises a mixture of a textile antistatic agent and 10 to 50 parts by weight of humectant. There may also be employed from 0.1 to about 1 part by weight of a nonionic or cationic type wetting agent to assist in dispersing of the antistatic composition. It is also preferable to incorporate in the coating composition from about 0.1 to about 1 part by weight of an electrolyte particularly if the humectant employed is nonionic in character or is only weakly ionic, i.e., has a relatively low dissociation constant. The antistatic coating is preferably applied in the form of an aqueous solution or dispersion, although other solvents or liquid dispersing mediums may be employed if desired and in the case of aqueous solutions or dispersions, volatile water-soluble solvents, such as lower aliphatic alcohols of one to four carbon atoms, acetone and the like, may be included to facilitate drying of the antistatic layer following its application.

A number of preferred compositions for the antistatic coating of the present invention are disclosed in

U.S. Pat. No. 3,519,561 of Andrew J. Kelly and Robert C. Britt entitled "Antistatic Composition and Process." Particularly preferred are those antistatic compositions disclosed in said patent in which potassium formate is employed as humectant since it has been found that not only is potassium formate particularly effective as a humectant in such coating compositions, but compositions containing the same are compatible with the latex backing where employed, in carpets, for instance, and specifically overcomes premature coagulation or gelling of the backing based on natural compounded rubber, thus not interfering with good bonding of the latex coating with the carpet backing. On the other hand, the antistatic coatings containing calcium chloride are incompatible with certain known latex coatings which have been used as carpet backings in that they cause premature coagulation or gelling of the latex with resultant poor adhesion of the latex to the carpet backing so that in the case of loosely woven or tufted carpets the latex does not function satisfactorily to hold the tufts in place. 15

While antistatic layers based on the antistatic compositions of the above mentioned patent are particularly preferred, it will be understood that one may also employ many antistatic materials in conjunction with the specific parameters of the instant invention. Such agents are normally nitrogen containing or carboxylic containing organic antistatic agents and as examples there may be mentioned the following compounds:

Bukester R1499 — lauric acid polyethylene glycol ester.

Amine oxides or quaternary ammonium salts of N-vinyl lactams, such as vinyl pyrrolidone-dimethylamino-ethylmethacrylate copolymers.

N-vinyl lactam acrylamine copolymers — such as a copolymer of 75% vinyl pyrrolidone and 25% acrylamide.

Zelex DP — lauryl alcohol phosphate.

Catanac SN — stearyl amidopropyl dimethyl- $\beta$ -hydroxyethyl ammonium nitrate.

Ethoquad C/12 — polyoxyethylated quaternary ammonium salt.

Phosphonamide sulfonate of an alcohol ethoxylate, i.e., a product of the formula



wherein R represents the hydrocarbon residue of an alkanol (such as Alfol (1412) and n represents an integer of 8 to 30.

Partial esters of the copolymer of vinyl methyl ether and maleic anhydride with nonionic surface active agents — described in French Pat. No. 1,360,209.

Esters of phosphoric acid and ethoxylated aliphatic alcohol, such as the phosphate esters of lauryl alcohol condensed with 4 moles of ethylene oxide or of dodecyl alcohol condensed with about 2 moles of ethylene oxide.

Polyglycol 4000

Sucrose octa-acetate

Polyethoxy amides of stearic and oleic acid

Methyl diethanolamine ethoxylate

Ethoxylated 2,3,7,9-tetramethyl-5-decyne-4,7-diol

Polyoxyethylenemono-oleate

Lauryl trimethyl ammonium chloride  
Undecylimidazolone  
Lauryl dimethylbenzyl ammonium chloride  
Polyoxyethyl stearyl ammonium chloride  
Oleic-monoisopropyl amide  
Vinyl acetate/styrene/acrylic acid polymers  
Ethoxylated diamines  
Long chain amine oxides



Hydroxybutyramides  
Quaternized polymers of vinylpyridine  
Quaternized copolymers of vinylpyridine and vinyl-pyrrolidone  
Phosphate esters of the type described in U.S. Pat. Nos. 3,004,056 and 3,004,057 and Belgian Pat. No. 641,097.

The phosphate esters of the type referred to in said patents may be prepared by reacting 1 mole of  $\text{P}_2\text{O}_5$  with 2 to 4.5 moles of a nonionic surface active agent having the molecular configuration of a condensation product of at least 1 mole of ethylene oxide with 1 mole of a compound containing at least six carbon atoms and a reactive hydrogen atom under substantially anhydrous conditions and at a temperature below about 110°C. The process does not require the use of an excess of the hydroxyl organic compound (in this instance the defined nonionic surface active agent), in order to bring the  $\text{P}_2\text{O}_5$  into solution. Substantially no tertiary phosphate ester is formed and little or no  $\text{P}_2\text{O}_5$  remains in the composition. Depending upon the particular ratio of  $\text{P}_2\text{O}_5$  to the nonionic surface active agent employed, and the nature of such nonionic, the product may in some instances contain some unreacted nonionic surface active agent which for certain uses is actually advantageous.

For similar reasons, the proportions of secondary phosphate ester:primary ester:free nonionic in the products thereof will in general fall within the range of about 20 to 45% secondary ester:30-80% primary ester:0-40% nonionic, by weight.

Lighter colored or substantially colorless products are obtained when the phosphorylation reaction is carried out in the presence of a small or catalytic amount of a phosphorus-containing compound selected from the group consisting of hypophosphorous acid, salts of hypophosphorous acid, phosphorous acid, and salts and esters of phosphorous acid. The process comprises reacting 1 mole of  $\text{P}_2\text{O}_5$  with 2 to 4.5 moles of a nonionic surface active agent having the molecular configuration of a condensation product of at least 1 mole of ethylene oxide with 1 mole of a compound containing at least 6 carbon atoms and a reactive hydrogen atom, under substantially anhydrous conditions and at a temperature below about 110°C. in the presence of a small amount of one or a mixture of the aforementioned hypophosphorous or phosphorous acid compounds.

By the use of such compounds in the described phosphorylation reaction, it has been found that an unexpected and substantial improvement in the (absence of) color of the products and the resistance of such products to discoloration in storage is obtained. Products resulting

from the use thereof generally have VCS (varnish color scale, Gardner scale, standards of 1933) values of at least one less than products of the same process carried out in the absence of the hypophosphorous or phosphorous acid compound. Products having a VCS color of about 1 or less are thus made possible, as compared with VCS colors of from about 2 to 7 or more for products produced without the aid of the present invention. Further, the products have been found to resist discolorations or darkening even after storage for 3 to 6 months.

The nonionic surface active agents employed as reactants are well known in the art and are disclosed along with suitable methods for their preparation in numerous patents and other publications. In general, they may be obtained by condensing a polyglycol ether containing the required number of alkenoxy groups or an alkylene oxide such as propylene oxide, butylene oxide, or preferably ethylene oxide, with an organic compound containing at least six carbon atoms and a reactive hydrogen atom. As such compounds containing a reactive hydrogen atom there may be mentioned alcohols, phenols, thiols, primary and secondary amines, and carboxylic and sulfonic acids, and their amides. The amount of alkylene oxide or equivalent condensed with the reactive chain, will depend primarily upon the particular compound with which it is condensed. As a convenient rule of thumb, an amount of alkylene oxide or equivalent should be employed which will result in a condensation product containing about 20 to 85% by weight of combined alkylene oxide. However, the optimum amount of alkylene oxide for attainment of the desired hydrophobic hydrophilic balance may be readily determined in any particular case by preliminary test and routine experimentation.

In general, the nonionic surface active agents, having the molecular configuration of a condensation product of at least 1 mole of an alkylene oxide, preferably ethylene oxide, with 1 mole of a compound containing at least six carbon atoms and a reactive hydrogen atom are preferably polyoxyalkylene derivatives of alkylated and polyalkylated phenols, multi-branched chain primary aliphatic alcohols having the molecular configuration of an alcohol produced by the Oxo process from a polyolefin of at least seven carbon atoms, and straight chain aliphatic alcohols of at least 10 carbon atoms. Examples of these derivatives and other suitable nonionic surface active agents which may be phosphated in accordance with the present invention are included below. In this list, "E.O." means "ethylene oxide" and the number preceding same refers to the number of moles thereof reacted with 1 mole of the given reactive hydrogen-containing compound.

Nonylphenol + 9-11 E.O.  
 Nonylphenol + 2 E.O.  
 Dinonylphenol + 7 E.O.  
 Dodecylphenol + 18 E.O.  
 Castor oil + 20 E.O.  
 Tall oil + 18 E.O.  
 Oleyl alcohol + 20 E.O.  
 Lauryl alcohol + 4 E.O.  
 Lauryl alcohol + 15 E.O.  
 Hexadecyl alcohol + 12 E.O.  
 Hexadecyl alcohol + 20 E.O.  
 Octadecyl alcohol + 20 E.O.  
 Oxo tridecyl alcohol:  
 (From tetrapropylene) + 7 E.O.

(From tetrapropylene) + 10 E.O.  
 (From tetrapropylene) + 15 E.O.  
 Dodecyl mercaptan + 9 E.O.  
 Soya bean oil amine + 10 E.O.  
 Rosin amine + 32 E.O.  
 Coconut fatty acid amine + 7 E.O.  
 Cocoa fatty acid + 10 E.O.  
 Dodecylbenzene sulfonamide + 10 E.O.  
 Decyl sulfonamide + 6 E.O.  
 Oleic acid + 5 E.O.  
 Polypropylene glycol (30 oxypropylene units) + 10 E.O.

In carrying out the phosphation reaction the  $P_2O_5$  is preferably added gradually, with vigorous agitation to the nonionic surface active agent in liquid form. If the latter agent is a solid at room temperature, it should be heated to above its melting point. Addition of the nonionic surface active agent to the  $P_2O_5$  is inadvisable since this has been found to result in the formation of tar and the like and to prevent the reaction from proceeding to completion. The reaction is exothermic and in some cases cooling is necessary to prevent the temperature from going above 110°C. since this tends to produce discolored and darkened products. The reaction proceeds continuously during addition of the  $P_2O_5$  and solution thereof in the nonionic surface active agent, and is substantially 90% complete or more by the time all of the  $P_2O_5$  has been added. The few particles of solid  $P_2O_5$  remaining in the reaction medium may be removed at this point if time is of the essence, but it is preferred in the interests of economy to allow the reaction to proceed for an additional period of time which may range from one-half to 5 hours or more at ambient temperatures up to about 110°C. until all of the  $P_2O_5$  has dissolved indicating complete reaction between the reactants involved. Vigorous agitation during the reaction is highly desirable to facilitate and expedite completion of the reaction.

It is an advantageous feature that the  $P_2O_5$  may be employed in dry, solid form as a granular powder or other finely divided or particulate form, for reaction with the above defined nonionic surface active agents. However, if desired, the  $P_2O_5$  may first be dispersed in an inert organic diluent such as benzene, xylene, ether, pentane, or low and high boiling hydrocarbon fractions.

After completion of the reaction, the reaction mixture may be cooled and discharged. If carried out under rigid anhydrous conditions the product should consist of a mixture of the primary and secondary phosphate esters of the nonionic surface active agent combined, depending upon the proportions of reactants, in some instances with a small proportion of unreacted nonionic surface active agent. Any small amount of water present in the reaction mixture will result protanto in the formation of some phosphoric acid in the product. The degree of esterification in the product may be determined by potentiometric titration or by titration with alkali to methyl orange and then to phenolphthalein.

The products may be supplied in free unneutralized form, or in the form of the partially or completely neutralized salts containing as cations alkali metals, alkaline earth metals, metals, ammonium and organic amines. It is to be understood that such salts are to be regarded as the equivalent of the present products in their free form. As examples of suitable cations, there

may be mentioned sodium, potassium, lithium, calcium, strontium, barium, magnesium, iron, tin, cadmium, aluminum, antimony, chromium, manganese, mercury, nickel, silver, zinc, ammonium and aliphatic, alicyclic, aromatic and heterocyclic organic amines such as the mono-, di- and tri-methylamines, ethylamines, propylamines, laurylamines, stearylamines, ethanolamines, propanolamines, butanolamines, hexanolamines, cyclohexylamines, phenylamines, pyridylamines, morpholinylamines, and the like.

Where desired, the above products may be modified by the addition to the reaction medium of a small amount of hypophosphorous or phosphorous acid compound. Generally, about 0.01 to 5% and preferably about 0.1 to 2% of such compound, based on the weight of the nonionic surface active agent being phosphated is sufficient to provide the desired improvements with respect to prevention of color degradation of the products and improvement in resistance of the products to color degradation in storage. Hypophosphorous acid and its alkali metal salts, e.g. sodium and potassium salts are generally preferred although any metal, alkaline earth metal, ammonium or amine salt of hypophosphorous acid or phosphorous acid may be employed, in addition to phosphorous acid per se. When hypophosphorous acid is employed, it is preferred to use a 30 to 50% aqueous solution thereof although aqueous solutions of this acid and other of the water soluble hypophosphorous and phosphorous acid compounds may be employed in the form of aqueous solutions ranging in concentration from less than 5 up to 70% or more. It should be borne in mind that the reaction should be carried out under substantially anhydrous conditions and accordingly the water introduced in such solutions should be held to a minimum.

The salts of hypophosphorous acid and phosphorous acid employed herein may be in their hydrated or dehydrated form. As examples of such salts, there may mentioned aluminum, cadmium, sodium, potassium, lithium, calcium, strontium, barium, magnesium, ammonium, mono-, di- and tri-methylamine, -ethylamine, -propylamine, -ethanolamine, and -propanolamine, pyridinyl, and morpholinyl phosphites and hypophosphites.

Esters of phosphorous acid may also be employed.

These esters may be described as mono-, di-, and tri-alkyl, -aryl, and -cycloalkyl phosphites. It will be understood that mixed esters are included. As some specific examples of such esters in which the esterifying group generally contains from about one to 20 carbon atoms, there may be mentioned ethyl phosphite, lauryl phosphite, Oxo tridecyl phosphite (the esterifying alcohol having the molecular configuration of an alcohol produced from tetrapropylene or triisobutylene by the Oxo process), stearyl phosphite, phenyl phosphite, cyclohexyl phosphite, the corresponding di- and tri-substituted phosphites, ethyl phenyl phosphite, ethyl diphenyl phosphite, lauryl cyclohexyl phosphite, dipropyl phenyl phosphite, and the like.

The hypophosphorous or phosphorous acid compound is preferably admixed with the non-ionic surface active agent prior to its addition to the nonionic surface active agent. It will accordingly be understood that the hypophosphorous or phosphorous acid compound or mixture thereof may be added at the start of the reaction or continuously or intermittently as the reaction proceeds.

The examples in the following table are only illustrative. In each of these examples, the nonionic surface active agent is first charged to a reactor equipped with an agitator. If the charge is solid at room temperature, it is heated to melt the same. The additive referred to in the table is then added to and dissolved in the non-ionic surface active agent with vigorous agitation. The solid granular  $P_2O_5$  is then charged to the reactor with vigorous agitation over a period ranging from about 5 minutes to about 1 hour and usually about 15 minutes. After the initial exothermic reaction subsides, the reaction mixture is heated to 100°C. and held at this temperature for about 5 hours after which the mixture is cooled and discharged. A sample of the reaction mixture is titrated with alkali to methyl orange and then to phenolphthalein as a control on the esterification. The VCS color readings are measured in the prescribed manner. A reading of one is the lowest color reading measurable by this method, the highest being 18. Products prepared with the use of the additives referred to in the table sustained no change in color after 3 to 6 months' storage.

Preferred are the monoesters, the diesters and the mixtures of same.

TABLE A

| Ex. | Nonionic agent                                             | Non-<br>ionic<br>parts | $P_2O_5$<br>parts | Parts   | Additive<br>where employed | VCS<br>Color |
|-----|------------------------------------------------------------|------------------------|-------------------|---------|----------------------------|--------------|
| 1   | Nonylphenol+2 E.O.<br>$C_9H_{19}C_6H_4(OC_2H_4)_2OH$       | 2,888                  | 284               | Control |                            | 2            |
| 2   | "                                                          | 2,288                  | 284               | 3.4     | Hypophosphorous acid (50%) | <1           |
| 3   | Nonylphenol+4 E.O.<br>$C_9H_{19}C_6H_4(OC_2H_4)_4OH$       | 2,855                  | 213               | Control |                            |              |
| 4   | "                                                          | 2,855                  | 213               | 4.2     | Hypophosphorous acid (50%) | <            |
| 5   | Nonylphenol+6 E.O.<br>$C_9H_{19}C_6H_4(OC_2H_4)_6OH$       | 484                    | 47.3              | Control |                            | 4            |
| 6   | "                                                          | 484                    | 47.3              | 1.0     | Hypophosphorous acid (50%) | <1           |
| 7   | "                                                          | 484                    | 47.3              | 0.5     | Sodium hypophosphite       | <1           |
| 8   | "                                                          | 484                    | 47.3              | 2.0     | Triphenyl phosphite        | 2            |
| 9   | Nonylphenol+10 E.O.<br>$C_9H_{19}C_6H_4(OC_2H_4)_{10}OH$   | 1,821                  | 108               | Control |                            | 4            |
| 10  | "                                                          | 1,821                  | 108               | 7.0     | Hypophosphorous acid (30%) | <1           |
| 11  | Nonylphenol+100 E.O.<br>$C_9H_{19}C_6H_4(OC_2H_4)_{100}OH$ | 605                    | 11.9              | Control |                            | 2            |
| 12  |                                                            | 605                    | 11.9              | 1.2     | Hypophosphorous acid (50%) | 1            |
| 13  | Dinonylphenol+7 E.O.<br>$C_{18}H_{35}C_6H_4(OC_2H_4)_7OH$  | 327                    | 23.6              | Control |                            | 5            |
| 14  | "                                                          | 327                    | 23.6              | 1.0     | Hypophosphorous acid (30%) | <1           |
| 15  | Dodecylphenol+6 E.O.<br>$C_{12}H_{25}C_6H_5(OC_2H_4)_6OH$  | 1,052                  | 94.4              | Control |                            | 4            |
| 16  | "                                                          | 1,052                  | 94.4              | 3.0     | Hypophosphorous acid (50%) | <1           |

TABLE A - Continued

| Ex. | Nonionic agent                                                                                                                    | Non-<br>ionic<br>parts | P <sub>3</sub> O <sub>5</sub><br>parts | Parts   | Additive<br>where employed | VCS<br>Color |
|-----|-----------------------------------------------------------------------------------------------------------------------------------|------------------------|----------------------------------------|---------|----------------------------|--------------|
| 17  | Oxo tridecyl alcohol <sup>1+</sup><br>3 E.O.<br>C <sub>13</sub> H <sub>27</sub> (OC <sub>2</sub> H <sub>4</sub> ) <sub>3</sub> OH | 166                    | 23.7                                   | Control |                            | 7            |
| 18  | "                                                                                                                                 | 166                    | 23.7                                   | 1.0     | Hypophosphorous acid (50%) | 2            |
| 19  | "                                                                                                                                 | 166                    | 23.7                                   | 1.0     | Phosphorous acid           | 2            |
| 20  | Lauryl alcohol+4 E.O.                                                                                                             | 724                    | 71                                     | Control |                            | 7            |
| 21  | C <sub>12</sub> H <sub>25</sub> (OC <sub>2</sub> H <sub>4</sub> ) <sub>3</sub> OH                                                 | 724                    | 71                                     | 1.8     | Hypophosphorous acid (50%) | 1            |

<sup>1</sup> From tetrapropylene by the Oxo process.

A suitable quaternary ammonium compound, may be represented by the following structural formula:



wherein R = —(CHY)<sub>n</sub>—CH<sub>3</sub> and n = 6 to 26; R'' & R' = —(CHY)<sub>n</sub>—CH<sub>3</sub> and n = 0 to 6. The alkyl moiety may be branched or straight chain, y being hydrogen or an alkyl group as defined above. R'' and R' need not be the same.

The quaternary ammonium compounds may be made in ways known in the art, such as for example by dissolving in isopropyl alcohol one mole of dimethyl stearyl amine; then from a separatory funnel add thereto one-half mole of diethyl sulfate keeping temperature below 50°C; after the last of the diethyl sulfate is added and the exotherm is stopped, reflux for 1 hour and cool. Evaporate the alcohol.

Preferred quaternary ammonium compounds include: compounds where R' and R'' are lower alkyl, particularly preferred is wherein R' or R'' are methyl. R may be C<sub>12-16</sub>, saturated or unsaturated, i.e., cocoa, stearic, oleic and the like.

The quaternized copolymers referred to may be those that are compounds which are first copolymerized and thereafter quaternized or those wherein the monomers are first quaternized and then copolymerized. Procedures known in the art for carrying out the above processes may be employed.

The quaternary copolymers employed are those which have unit I and either unit II or III or all three units.



wherein n represents 40 - 90 mole percent, m is 10 - 60 mole percent, p is from 10 - 60 mole percent, and n + m or p = 100; or n + (m + p) = 100; R<sub>1</sub> is H or CH<sub>3</sub>; R<sub>2</sub> is

or C<sub>x</sub>H<sub>2</sub> where x = 2-18; R<sub>3</sub> is CH<sub>3</sub> or C<sub>2</sub>H<sub>5</sub>; R<sub>4</sub> is CH<sub>3</sub>, C<sub>2</sub>H<sub>5</sub>,



X is Cl, Br, I, SO<sub>4</sub>, HSO<sub>4</sub>, CH<sub>3</sub>SO<sub>3</sub>; and M is a monomeric unit resulting from the heteropolymerization employing an optional mono vinyl monomer different from and copolymerizable with n. M may also be 5 to 40 where p is 0 to 50, the latter occurring where n, m and p are all employed.

As indicated from the above formula, such quaternary copolymers are prepared by the copolymerization of an N-vinyl lactam, such as N-vinyl pyrrolidone and di-loweralkylaminoalkyl (or hydroxy alkyl) acrylate or methacrylate, and optionally a further mono vinyl monomer different from and copolymerizable with n. The monomers are copolymerized in accordance with the present invention so that based upon 100 mole percent, the vinyl pyrrolidone units are present in an amount of 40 - 90 mole percent, the units derived from the diloweralkylaminoalkyl (or hydroxy alkyl) acrylate or methacrylate constitute from 10 to 60 mole percent, and the units derived from said further copolymerizable vinyl monomer also constitute from 10 to 60 mole percent.

The polymeric N-vinyl lactams utilized in the preparation of the compositions of this invention are characterized by the following general structural formula:



III



wherein R represents an alkylene bridge group necessary to complete a five, six or seven-membered heterocyclic ring system, R' represents either hydrogen or a methyl group, and n represents a number indicative of

the extent of polymerization and is usually at least 3 or 4.

All of the specific polymeric materials characterized by the foregoing general formula are commercially available and called polymeric N-vinyl lactams. They are obtained by polymerizing organic five, six or seven-membered ring compounds containing in their rings the —NH-CO-group, such as, for example,

N-vinyl-2-pyrrolidone,  
N-vinyl-2-piperidone,  
N-vinyl-2-caprolactam,  
N-vinyl-3-methyl-2-pyrrolidone,  
N-vinyl-3-methyl-2-piperidone, or  
N-vinyl-3-methyl-2-caprolactam,  
N-vinyl-4-methyl-2-pyrrolidone,  
N-vinyl-4-methyl-2-piperidone or  
N-vinyl-4-methyl-2-caprolactam,  
N-vinyl-5-methyl-2-pyrrolidone,  
N-vinyl-5-methyl-2piperidone,  
N-vinyl-3-methyl-2pyrrolidone,  
N-vinyl-4,5-dimethyl-2-pyrrolidone,  
N-vinyl-5,5-dimethyl-2-pyrrolidone,  
N-vinyl-3,3,5-trimethyl-2-pyrrolidone,  
N-vinyl-5-methyl-5-ethyl-2-pyrrolidone,  
N-vinyl-3,4,5-trimethyl-3-ethyl-2-pyrrolidone,  
N-vinyl-6-methyl-2-piperidone,  
N-vinyl-6-ethyl-2-piperidone,  
N-vinyl-3,5-dimethyl-2-piperidone,  
N-vinyl-4,4-dimethyl-2-piperidone,  
N-vinyl-7-methyl-2-caprolactam,  
N-vinyl-7-ethyl-2-caprolactam,  
N-vinyl-3,5-dimethyl-2-caprolactam,  
N-vinyl-4,6-dimethyl-2-caprolactam and  
N-vinyl-3,5,7-trimethyl-2-caprolactam.

Of these several compounds, N-vinyl-2-pyrrolidone is most preferred as it is readily available and provides products having excellent properties.

Exemplary di-loweralkylaminoalkyl (or hydroxy alkyl) acrylates or methacrylates suitably employed include such materials as:

dimethylaminomethyl acrylate  
dimethylaminomethyl methacrylate  
diethylaminomethyl acrylate  
diethylaminomethyl methacrylate  
dimethylaminoethyl acrylate  
dimethylaminoethyl methacrylate  
dimethylamino-2-hydroxy propyl acrylate  
dimethylamino-2-hydroxy propyl methacrylate  
diethylamino-2-hydroxy ethyl acrylate  
diethylamino-2-hydroxy ethyl methacrylate  
dimethylaminobutyl acrylate  
dimethylaminobutyl methacrylate  
dimethylaminoamyl methacrylate  
diethylaminoamyl methacrylate  
dimethylaminohexyl acrylate  
diethylaminohexyl methacrylate  
dimethylaminooctyl acrylate  
dimethylaminoctyl methacrylate  
diethylaminoctyl acrylate  
diethylaminoctyl methacrylate  
dimethylaminodecyl methacrylate  
dimethylaminododecyl methacrylate  
diethylaminolauryl acrylate  
diethylaminolauryl methacrylate  
dimethylaminostearyl acrylate  
dimethylaminostearyl methacrylate  
diethylaminostearyl acrylate

diethylaminostearyl methacrylate  
etc. the non-hydroxy alkyl units being preferred.

The optional mono vinyl or vinylidene monomer represented by M in the above structural formula can comprise any conventional vinyl monomer copolymerizable with N-vinyl pyrrolidone. Thus, for example, suitable conventional vinyl monomers include the alkyl vinyl ethers, e.g., methyl vinyl ether, ethyl vinyl ether, octyl vinyl ether, etc.; acrylic and methacrylic acid and esters thereof, e.g., methacrylate, methyl methacrylate, etc.; vinyl aromatic monomers, e.g., styrene,  $\alpha$ -methyl styrene, etc.; vinyl acetate; vinyl alcohol; vinylidene chloride; acrylonitrile and substituted derivatives thereof; methacrylonitrile and substituted derivatives thereof; 15 acrylamide and methacrylamide and N-substituted derivatives thereof; vinyl chloride, crotonic acid and esters thereof; etc. Again, it is noted that such copolymerizable vinyl monomers can comprise any conventional vinyl monomer copolymerizable with N-vinyl pyrrolidone and where a terpolymer is formed, copolymerizable with both units *n* and *m*, and being different from both.

Accordingly, the preferred quaternized copolymers employed in the present invention can be characterized as having a repeating structural unit derived from

- A. 40 - 90 mole % of vinyl lactam;
- B. 10 - 60 mole % of a di-loweralkylaminoalkyl acrylate or methacrylate of a di-loweralkylaminohydroxyalkyl acrylate or methacrylate; or
- 30 C. 10 - 60 mole % of a vinyl monomer different from and copolymerizable with A and B.

Such copolymers are conveniently prepared by subjecting a solution of vinyl lactam and the amino acrylate or amino methacrylate monomer with or without an optional copolymerizable vinyl monomer to conditions conducive to vinyl polymerization through the double bond. Thus, for example, polymerization may suitably be initiated by the action of free radicals, the polymerization proceeding exothermically once initiated. Suitable free radical catalysts conveniently employed and suitably utilized in accordance with the production of the copolymers include organic and inorganic peroxides, e.g., hydrogen peroxide, t-butyl peroxide, etc., aliphatic azo compounds, e.g., azobisisobutyronitrile as well as other free radical forming catalysts well known in the polymerization art.

The polymerization is preferably carried out in solution at temperatures varying from about 50°C to 100°C or more; however, to avoid run away conditions and to obtain a copolymer of a desirable molecular weight it is sometimes preferred to carry out the copolymerization at a temperature of from about 75 to about 85°C. The copolymerization reaction is preferably carried out in the absence of free-oxygen, conveniently under a blanket of an inert gas, such as, nitrogen, argon or the like, or at atmospheric pressure.

As indicated previously the copolymers are in the form of their quaternary salts. Accordingly, after completion of the polymerization reaction the polymer is submitted to a treatment conducive to quaternization of the tertiary amino group, utilizing a conventional quaternizing agent. Thus, noting the above structural formula for the copolymers, suitable quaternizing agents include, such as, dialkyl sulfates, e.g., dimethyl sulfate, diethyl sulfate, etc.; alkyl sulfonic acid, e.g., methyl sulfonic acid, ethyl sulfonic acid, ethyl sulfonic acid, etc.; benzyl halides, e.g., benzyl chloride, benzyl



gredients are preferably prepared in the form of an aqueous liquid fluid medium so that they can be applied to the material to be protected in the form of an aqueous solution, dispersion, gel, viscous mass or the like.

The composition of the present invention comprises a mixture of the above components in the following relative proportions in which the parts are by weight. For each part of alkoxylated amine there is used from equivalent amounts to about 5 parts of humectant. If the particular humectant employed is also a strong electrolyte the amount employed as a humectant is sufficient to function as an electrolyte. However, if the particular humectant is not a strong electrolyte then from 0.01 part to about 0.01 part of a strong electrolyte is employed. Both components are prepared in the form of a concentrated aqueous solution or dispersion.

It is of course within the purview of the invention to add to the composition, compatible materials which do not affect the basic and novel characteristics thereof. Among such materials are wetting agents of the non-ionic or cationic type. Such wetting agents may be used in amounts of from 0.01 to 0.1 part by weight and are preferably included in the composition when a heavy pile fabric, particularly carpeting is being treated, as they facilitate the penetration of the antistatic composition into the textile substrate where so desired. It is preferable to add a measured amount of wetting agent as determined by preliminary test, to control the degree of penetration of the composition into the textile substrate when same is desired, particularly when treating carpet so that the composition penetrates the backing of carpet and wets the base of the pile fabric, but does not penetrate to the outer tips of the pile. Where the antistatic composition will not penetrate the backing of the carpet, the use of the wetting agent is not as important. Other materials which can be incorporated in the composition include coloring agents, including dyes and pigments, fillers and similar additives, antioxidants, additional antistatic agents, stabilizers and defoaming agents. There may also be incorporated various volatile water soluble solvents, such as lower alcohols of one to four carbon atoms, acetone and the like in order to facilitate the removal, by vaporization, of excess water.

The antistatic coating composition of the present invention is prepared by dissolving the several components, alkoxylated amine, combined humectant and electrolyte or humectant and an electrolyte in water, the order of addition being immaterial and mixing at from room temperature to about 100°C for a sufficient length of time until a uniform composition is obtained. When a salt of a lower carboxylic acid is employed as the humectant or combined humectant and electrolyte, it may be formed in situ by adding carboxylic acid having from about one to about five carbon atoms and an alkali metal or alkaline earth metal base, i.e., hydroxide or carbonate, such as sodium, potassium lithium or cesium hydroxide or carbonate.

After all the components are added to water and a uniform mix is obtained, the pH of the resulting mixture or solution is adjusted so as to be within the range of pH 7 to 13, more preferably to a pH within the range of from about 9 to about 11, with the most preferred pH being about 9. This pH adjustment is preferably effected by adding an alkali or an organic amine to the mixture and if the alkali salt of a lower carboxylic acid is employed as humectant and/or electrolyte, it is pref-

erable that the pH adjustment be effected using the same alkali base as the anion present in such salt. It will be appreciated that this pH adjustment by addition thereof also results in the formation of a salt of the alkoxylated amine.

As neutralizing agents there may be employed alkalies, such as, KOH, NaOH, Ca(OH)<sub>2</sub>, Na<sub>2</sub>CO<sub>3</sub>, ammonia, diethanol amine, triethanol amine, morpholine and other organic amines and the like.

Subsequent to neutralizing the antistatic composition, the latter may be thickened or made viscous by the addition thereto of .1 to 20% by wt. of common thickness such as, sodium polyacrylates; acrylic acid; methyl cellulose, hydroxy ethyl cellulose; starch and the like.

The antistatic composition of the present invention is particularly useful for the production of the antistatic textile products described and claimed in U.S. Pat. Nos. 3,510,386 and 3,519,561 both of which also more fully describes the preferred method of application. However, for the sake of a complete disclosure the preferred method of application of the antistatic composition of the present invention to textiles is illustrated diagrammatically in the annexed sheet of drawings; in which 2 designates a roll of textile material, such as carpeting or upholstery, preferably of pile construction, to be treated. The web of textile 4 which may contain a polymeric latex pre-coat over the primary backing is removed from the roll by drive rollers 14 and passes over coating means 6, here illustrated as a spray head which applies the coating composition to the back of the textile, to the underside of the primary backing or that of the latex pre-coat. The web of textile then passes through drying unit 8 illustrated diagrammatically in the drawing as a drying oven, wherein it may be subjected to radiant heat and/or heated atmosphere to effect evaporation of most of the water. It will be apparent that due to the evaporation of water, the temperature of the surface of the textile will not exceed 212°F., but a surrounding atmosphere having temperatures of from 300° to 400°F may be employed subject to the practical limitation that the temperature must not be so high as to affect decomposition or degradation of the textile substrate (latex pre-coat) or the antistatic coating composition. When essentially all of the water has been removed by vaporization, the web of textile then passes through suitable apparatus illustrated in the drawings as coating roll 10 for applying a latex backing to the fabric. In the case of a loosely woven or tufted carpet structure the latex backing is applied in the manner customary in the art so as to assure uniform coating and good adhesion of the latex to the backing and looped ends of the pile. Any conventional latex backing may be employed, particularly preferred is the compounded natural rubber latexes, such as Lotol GX-1314. There may also be used compounded neoprene latexes, such as Lotol GX-1076 and latexes of polystyrene, vinylidene chloride polyacrylates, butadiene-styrene or others.

The antistatic composition can be applied in any coating weight which is capable of effecting the desired antistatic properties. For use on carpets the broad dry coating weight range is from .01 to 20 oz. per sq. yd. with a more preferred range being 2.0 to 10 oz. per sq. yd. A more preferred dry coating weight for carpet is 4-6 oz. per sq. yd. For application on conventional textiles such as woven fabrics the broad dry coating weight

range is from above 10% to about 4.0% based on fabric weight. A more preferred dry coating range for textiles is from about 0.8% to about 3.0% based on fabric weight. A most preferred dry coating weight for textiles is 2.0% based on fabric weight.

The details of the present invention will be apparent to those skilled in the art from a consideration of the following specific examples and claims in which the parts, proportions and percentages are by weight, unless otherwise noted.

#### EXAMPLES 1-24

In these examples the antistatic composition was prepared by adding the base and organic acid to water to form the humectant in situ. The alkoxylated amine employed was stearyl amine which had been ethoxylated with 20 moles of ethylene oxide per mole of amine. The wetting agent when employed was tridecyl alcohol which had been ethoxylated with 6 moles of ethylene oxide per mole of alcohol. The thus prepared antistatic composition is then neutralized with 45% alkali (i.e., KOH) to a pH of 6.0-8.0. This neutralization is then continued to a pH of 9-13 by employing an amine (i.e., triethanol amine). Where it is desired to thicken the antistatic composition, same may be carried out either to the exclusion of raising the pH thereof or in addition thereto by adding to the composition .1 to 10% by weight, preferably .2 to 2% of one of said thickening agents. The amounts of materials employed in each example are given in the appropriate column of Table I.

In most examples the antistatic coating was applied to the back of a tufted carpet having a primary loosely woven jute backing rather than to the underside of a pre-coat latex; the type of fibers employed in the tufted pile are given in Table I as well as the amount of antistatic composition applied. After application of the antistatic coating the carpet was dried to remove excess moisture. A latex coating was then applied over the antistatic coating in such a manner that it did not encapsulate the latter where no polymeric pre-coat latex had been employed.

The testing procedure used in these examples was the AATC-134-1969 Test.

#### EXAMPLE I

The acidic antistatic composition (pH 4-7) was neutralized with 45% KOH to 6.0-6.5 pH. This neutralization was continued with triethanol amine to pH 9.0. The thus neutralized antistatic composition was applied to the back of a tufted carpet of plush style with nylon face yarn and a woven polypropylene primary backing by roller coating. Wet application weights of 5.2 oz. per sq. yd. were achieved (determined by a chloride ion determination). The treated carpet was dried and subsequently laminated to jute using an adhesive compound consisting of carboxylated styrene-butadiene latex loaded to 350 parts with whiting. Static test results by AATC-134-1969 at 20% relative humidity were taken. Untreated carpet under same AATC-134-1969 test procedure were also taken. The results appear in Table I. The threshold for human shock sensitivity is generally accepted as + or -2,800 volts by this test procedure.

#### EXAMPLE II

The acidic antistatic composition was neutralized to pH 9.0 with KOH and applied to a shag carpet with nylon face yarn and polypropylene backing. The com-

position was applied to back of the lock of the carpet at various wet application levels, dried and laminated to a jute secondary backing with a natural latex adhesive.

5

#### EXAMPLE III

Carbon steel coupons were placed in the neutralized antistatic composition of Examples I and II along with the unneutralized antistatic composition. Test results 10 were as follows:

|                                             |                                                |
|---------------------------------------------|------------------------------------------------|
| neutralized to pH 9.0 with triethanol amine | No corrosion after 1 week at room temperature  |
| neutralized to pH 9.0 with KOH              | No corrosion after 2 weeks at room temperature |
| control of pH 6.3                           | Corrosion noticeable after 3 hours.            |

#### EXAMPLE VI

20 A nylon fine plush carpet with a woven polypropylene primary backing was coated with 28 ounces per sq. yd. of 15% thickened antistatic composition to 12,000 cps with Union Carbide "Cellosize QP 100M" (Brookfield RVF No. 6-10 RPM) and dried. Carpet so treated exhibited a reduced tendency to migration of the antistatic component to the face either after shampooing or 25 after soaking in water.

#### EXAMPLE V

30 Example IV was repeated except that a secondary jute backing was applied. Substantially the same results were obtained.

#### EXAMPLE VI

35 Example IV was repeated using a woven carpet consisting primarily of wool fibers. Substantially the same results were obtained.

#### EXAMPLE VII

40 A thickened antistatic medium (400 cps LVF-Spindle No. 3, speed 10) was prepared and employed on a shag carpet that had exhibited migration problems. There was no evidence of migration on the carpet after treatment.

#### EXAMPLE VIII

45 Example IV was repeated except that an unthickened antistatic composition was used. Substantial migration to the surface took place after shampooing and soaking in water.

#### EXAMPLE IX

50 Example IV was repeated but at 2,000 cps (Brookfield LVF No. 3 at 12 RPM). Substantially no antistatic composition migrated to the surface after shampooing and soaking in water.

#### EXAMPLE X

55 Example IV was repeated but at 500 cps (Brookfield LVF No. 3 at 12 RPM). Migration of antistatic composition to the surface was substantially reduced as compared to the standard antistatic composition having a viscosity of 5 cps (Brookfield LVF No. 1 at 60 RPM).

#### EXAMPLES 24 to 41

60 In these examples the samples treated were nylon and wool tufted carpet structures. In most cases the antistatic coating was applied to the base of the carpet fibers

and primary jute and dried. A latex coating was then applied over the antistatic coating.

In these examples the humectant was formed in situ by the reaction of a basic component with an acidic component. The amine and wetting agent were the same as previously described.

The composition of the antistatic coating, as well as the test results and other pertinent information for these examples are given in Table II and IV.

#### EXAMPLES 42 to 56

In these examples the samples treated were nylon and wool tufted carpet structures. In most cases the antistatic coating was applied to the base of the carpet fibers and primary jute backing and dried to remove the excess moisture. In these examples the wetting agent utilized was in accordance with the description given in regard to Examples 1 to 25.

In these examples the humectant was not formed in situ but instead was added directly to the antistatic composition. In Examples 48-51 the calcium chloride functioned as both a humectant and electrolyte.

The composition of the antistatic coating as well as the test results and other pertinent information for these examples are given in Tables V & VI.

#### EXAMPLES 57-83

In these examples the samples treated were conventional woven and nonwoven fabrics. In most cases the antistatic coating was applied to the textile and dried to remove the excess moisture. The amine utilized was in accordance with the description given in accordance with Examples 1 to 25. In these examples a wetting agent was not utilized.

In these examples the humectant was formed in situ by the reaction of a basic component with an acidic component as in Examples 1-25. The procedure for these examples was as follows: The samples were cut and coated with the antistatic coating. In these examples the coating weight was based on the weight of the fabric in question. A polymeric backing was then ap-

plied to the fabric and dried at a temperature of from about 200° to 325°F for a period of time of from about 10 to 30 minutes. The dried fabric was then conditioned for at least 6 hours at a temperature of 70°±5°F and 35 to 40% relative humidity. The coated material was then tested on an Atlab tester, as developed by the Atlas Chemical Co., Wilmington, Del. The test procedure consists essentially of a means of controlled rubbing of a strip of fabric across a pair of static-generating (Teflon) bars and across a stainless steel bar which transfers the friction generated charge to an electrostatic voltmeter for measurement. This testing was conducted at 77°F ± 2°F and at a constant relative humidity of 35 to 40%.

The composition of the antistatic coating, as well as the test results and other pertinent information for these examples, are given in Table VII.

#### EXAMPLES 85-113

In these examples the samples treated were conventionally woven and nonwoven fabrics of the type and fibers shown in Table IX. In most cases the antistatic coating was applied to the back of the textile sample and dried to remove excess moisture. A polymeric backing was then applied to the fabric and cured at a temperature of from 200°-235°F for from 10-30 minutes. The coated material was then tested on an Atlab Tester in the manner described above in connection with Examples 57-83. In these examples the humectant was not formed in situ, but instead was added directly to the antistatic composition.

The composition of the antistatic coating as well as test results and other pertinent data for these examples are given in Table VIII.

#### EXAMPLES 114-123

In these examples the flooring was treated in accordance with the information outlined in Table IX. The electrostatic test results of the treated flooring is given in Table X.

TABLE I

| Ex.<br>No.      | Basic<br>Com-<br>pound | Humectant |                 |                | Parts<br>Wetting<br>Agent | Electro-<br>lyte | Parts<br>Water | pH<br>Adjustment<br>Acid or Base | pH  | Carpet<br>Fiber    | Coating<br>wt. in<br>ozs. per<br>sq. yard |               |         |
|-----------------|------------------------|-----------|-----------------|----------------|---------------------------|------------------|----------------|----------------------------------|-----|--------------------|-------------------------------------------|---------------|---------|
|                 |                        | Parts     | Organic<br>Acid | Parts<br>Amine |                           |                  |                |                                  |     |                    |                                           |               |         |
| 1               | NaOH                   | 40        | Acetic          | 60             | 20                        | 2                | NaCl           | 2                                | 210 | KOH                | 9                                         | Nylon         | 5.2     |
| 2               | NaOH                   | 40        | "               | 60             | 20                        | 2                | NaCl           | 2                                | 210 | KOH                | 9                                         | Nylon         | 4-6 oz. |
| 3               | NaOH                   | 56        | Formic          | 46             | 20                        | 2                | NaCl           | 2                                | 180 | TRIETA             | 9                                         | Nylon         | 5.4     |
| 4               | NaOH                   | 40        | Acetic          | 60             | 20                        | 2                | NaCl           | 2                                | 210 | NaOH               | 8                                         | Nylon         | 4       |
| 5               | NaOH                   | 40        | "               | 60             | 20                        | 2                | NaCl           | 2                                | 210 | NaOH               | 8                                         | Wool          | 4       |
| 6               | KOH                    | 56        | Formic          | 46             | 20                        | 2                | NaCl           | 2                                | 180 | NaOH               | 9                                         | Nylon         | 4       |
| 7               | KOH                    | 56        | "               | 46             | 20                        | 2                | NaCl           | 2                                | 180 | NaOH               | 9                                         | Wool          | 4       |
| 8               | NaOH                   | 20        | "               | 23             | 10                        | 1                | KCl            | 1                                | 150 | NaOH               | 10                                        | Nylon         | 6       |
| 9               | NaOH                   | 20        | "               | 23             | 10                        | 1                | KCl            | 1                                | 150 | NaOH               | 10                                        | Wool          | 6       |
| 10              | KOH                    | 56        | Acetic          | 60             | 20                        | 2                | NaCl           | 2                                | 200 | NaOH               | 11                                        | Nylon         | 4       |
| 11              | KOH                    | 56        | Acetic          | 60             | 20                        | 2                | NaCl           | 2                                | 200 | NaOH               | 11                                        | Wool          | 4       |
| 12              | KOH                    | 56        | "               | 74             | 25                        | 2                | NaCl           | 3                                | 500 | NaOH               | 12                                        | Nylon         | 4       |
| 13              | KOH                    | 56        | "               | 74             | 25                        | 2                | NaCl           | 3                                | 500 | NaOH               | 12                                        | Wool          | 4       |
| 14              | KOH                    | 69        | Formic          | 56             | 25                        | 3                | NaCl           | 2.5                              | 245 | KOH                | 12                                        | Nylon         | 4       |
| 15              | KOH                    | 69        | "               | 56             | 25                        | 3                | NaCl           | 2.5                              | 245 | KOH                | 12                                        | Wool          | 4       |
| 16 <sup>1</sup> |                        |           |                 |                |                           |                  |                |                                  |     |                    |                                           | Nylon         |         |
| 17 <sup>1</sup> |                        |           |                 |                |                           |                  |                |                                  |     |                    |                                           | Wool          |         |
| 18              | KOH                    | 56        | Formic          | 56             | 20                        | 2                | NaCl           | 2                                | 150 | KOH                | 9                                         | Acrylic       | 4       |
| 19              | KOH                    | 56        | "               | 56             | 20                        | 2                | NaCl           | 2                                | 150 | KOH                | 9                                         | Polyester     | 4       |
| 20              | KOH                    | 56        | "               | 56             | 20                        | 2                | NaCl           | 2                                | 150 | KOH                | 9                                         | Polypropylene | 4       |
| 21              | KOH                    | 56        | "               | 56             | 20                        | 2                | NaCl           | 2                                | 150 | NH <sub>4</sub> OH | 9                                         | Nylon         | 4       |
| 22              | KOH                    | 56        | "               | 56             | 20                        | 2                | NaCl           | 2                                | 150 | Dietanol amine     | 9                                         | Nylon         | 4       |
| 23              | KOH                    | 56        | "               | 56             | 20                        | 2                | NaCl           | 2                                | 150 | Morpholene         | 9                                         | Nylon         | 4       |
| 24              | KOH                    | 56        | "               | 56             | 20                        | 2                | NaCl           | 2                                | 150 | TEA                | 9                                         | Nylon         | 4       |

<sup>1</sup>Untreated control.

TABLE IA — FLAMMABILITY IMPROVEMENT

Experiment No. 18 was thickened to 2,000 cps with .8% ethyl-cellulose. The thus treated material and the untreated material of Experiment 18 were then both applied at 6 ozs. to the back of a nylon, shag carpet with a loose twist of 48 ozs. faceweight nylon. The material was dried and a latex adhesive compound was applied on the back in the conventional way and jute backing applied. It was then dried and thereafter cured.

Part of each sample was shampooed with a sodium lauryl sulfate shampoo and a commercial home shampoo.

The samples were tested for flammability by the DOC-FF-1-70 Test.

|    | SAMPLE                                      | NUMBER OF PASS | NUMBER OF FAILURE |
|----|---------------------------------------------|----------------|-------------------|
| 5  | Experiment No. 18- 6 oz/sq. yd.             | 8              | 0                 |
|    | Experiment No. 18- 6 oz/sq. yd.<br>2000 cps | 8              | 0                 |
|    | After shampooing                            |                |                   |
| 10 | Experiment No. 18- 6 oz/sq. yd.             | 0              | 8                 |
|    | Experiment No. 18- 6 oz/sq. yd.<br>2000 cps | 8              | 0                 |

TABLE II

## STATIC RESULTS ACCORDING TO AATC 134-1969

| Ex. | Before Cleaning |               | After Steam Cleaning |            | Control - No Treatment |                   |
|-----|-----------------|---------------|----------------------|------------|------------------------|-------------------|
|     | Chrome Leather  | Neolite       | Chrome Leather       | Neolite    | Chrome Leather         | Neolite           |
| 1   | +1000 Volts     | +1300 Volts   | 1000 Volts           | 1100 Volts | +9,000 Volts           | -4 to 5,000 Volts |
| 2   | -1500 to -500   | -800 to -1200 | 850                  | 700        | +9,000-10,000          | -5,000 to 8,000   |
| 3   | 1100            | 1200          | 900                  | 1000       |                        |                   |
| 4   | 1100            | 900           | 800                  | 700        |                        |                   |
| 5   | 1300            | 1100          | 700                  | 900        |                        |                   |
| 6   | 1000            | 1100          | 1,100                | 1000       |                        |                   |
| 7   | 700             | 1000          | 600                  | 800        |                        |                   |
| 8   | 1200            | 1300          | 500                  | 500        |                        |                   |
| 9   | 900             | 1200          | 800                  | 900        |                        |                   |
| 10  | 800             | 700           | 700                  | 500        |                        |                   |
| 11  | -1100 -900      | -700 -1200    | 900                  | 1000       |                        |                   |
| 12  | 1200            | 1100          | 800                  | 1000       |                        |                   |
| 13  | 500             | 700           | 300                  | 400        |                        |                   |
| 14  | 800             | 900           | 710                  | 200        |                        |                   |
| 15  | 1100            | 1000          | 700                  | 900        |                        |                   |
| 16  | 1200            | 1000          | 700                  | 900        |                        |                   |
| 17  | 1100            | 1000          | 1200                 | 900        |                        |                   |
| 18  | 200             | 100           | 100                  | 200        | 11,000                 | 6,000             |
| 19  | 300             | 200           | 200                  | 300        | 7,000                  | 3,000             |
| 20  | 100             | 200           | 200                  | 400        | 9,000                  | 5,000             |
| 21  | 1100            | 1200          | 1000                 | 1200       |                        |                   |
| 22  | 800             | 1100          | 800                  | 1000       |                        |                   |
| 23  | 700             | 800           | 500                  | 700        |                        |                   |
| 24  | 1200            | 1000          | 800                  | 800        |                        |                   |

TABLE III

| Ex. | Humectant              |          |           |      | Parts<br>Wetting | Electro-<br>lyte | Parts<br>Water | pH<br>Adjustment<br>Acid<br>or Base | Carpet | Fiber              | Coating<br>wt.in<br>ozs.per<br>sq.yard |  |  |  |  |
|-----|------------------------|----------|-----------|------|------------------|------------------|----------------|-------------------------------------|--------|--------------------|----------------------------------------|--|--|--|--|
|     | Basic                  |          | Organic   |      |                  |                  |                |                                     |        |                    |                                        |  |  |  |  |
|     | No.                    | Compound | Parts     | Acid | Parts            | Amine            | Agent          |                                     |        |                    |                                        |  |  |  |  |
| 25  | NaOH                   | 40       | Acetic    | 60   | 20               | 2                | NaCl           | 2                                   | 210    | Trethanol<br>amine | 8                                      |  |  |  |  |
| 26  | NaOH                   | 40       | do.       | 60   | 20               | 2                | NaCl           | 2                                   | 210    | do.                | 10                                     |  |  |  |  |
| 27  | KOH                    | 56       | Formic    | 46   | 20               | 2                | NaCl           | 2                                   | 180    | Diethanol<br>amine | 8                                      |  |  |  |  |
| 28  | KOH                    | 56       | do.       | 46   | 20               | 2                | NaCl           | 2                                   | 180    | do.                | 9                                      |  |  |  |  |
| 29  | NaOH                   | 20       | do.       | 23   | 10               | 1                | KCl            | 1                                   | 150    | do.                | 10                                     |  |  |  |  |
| 30  | NaOH                   | 20       | do.       | 23   | 10               | 1                | KCl            | 1                                   | 150    | do.                | 12                                     |  |  |  |  |
| 31  | KOH                    | 56       | Acetic    | 60   | 20               | 2                | NaCl           | 1                                   | 200    | NH <sub>4</sub> OH | 10                                     |  |  |  |  |
| 32  | KOH                    | 56       | do.       | 60   | 20               | 2                | NaCl           | 1                                   | 200    | do.                | Wool                                   |  |  |  |  |
| 33  | KOH                    | 56       | Propionic | 74   | 25               | 2                | NaCl           | 3                                   | 500    | KOH                | 8                                      |  |  |  |  |
| 34  | KOH                    | 56       | do.       | 74   | 25               | 2                | NaCl           | 3                                   | 500    | do.                | 8                                      |  |  |  |  |
| 35  | KOH                    | 69       | Formic    | 56   | 25               | 3                | NaCl           | 2.5                                 | 245    | do.                | 8                                      |  |  |  |  |
| 36  | KOH                    | 69       | do.       | 56   | 25               | 3                | NaCl           | 2.5                                 | 245    | do.                | 8                                      |  |  |  |  |
| 37  | 29% NH <sub>4</sub> OH | 121      | Acetic    | 60   | *20              | 2                | NaCl           | 2                                   | 200    | NH <sub>4</sub> OH | 8                                      |  |  |  |  |
| 38  | 29% NH <sub>4</sub> OH | 121      | Formic    | 46   | 20               | 2                | NaCl           | 2                                   | 200    | do.                | 8                                      |  |  |  |  |
| 39  | 29% NH <sub>4</sub> OH | 121      | Propionic | 74   | 20               | 2                | NaCl           | 2                                   | 400    | do.                | do.                                    |  |  |  |  |
| 40' |                        |          |           |      |                  |                  |                |                                     |        |                    | Wool                                   |  |  |  |  |
| 41' |                        |          |           |      |                  |                  |                |                                     |        |                    |                                        |  |  |  |  |

\*Untreated control

\*Quaternized ammonium sulfate

TABLE IV

#### STATIC RESULTS ACCORDING TO AATC 134-1969

| Ex. | Before Cleaning |         | After Steam Cleaning |         |
|-----|-----------------|---------|----------------------|---------|
|     | Chrome Leather  | Neolite | Chrome Leather       | Neolite |
| 25  |                 |         |                      |         |
| 26  | 1200            | 900     | 1400                 | 1000    |
| 27  | 900             | 1200    | 1100                 | 1100    |
| 28  | 1500            | 1200    | 1200                 | 1500    |
| 29  | 1200            | 1400    | 1100                 | 1700    |
| 30  | 1400            | 1100    | 1200                 | 1200    |
| 31  | 900             | 700     | 800                  | 1000    |
| 32  | 1600            | 1200    | 1500                 | 1100    |
| 33  | 1400            | 1100    | 1600                 | 1500    |
| 34  | 1700            | 1700    | 2000                 | 2000    |
| 35  | 1600            | 1700    | 1900                 | 1800    |
| 36  | 600             | 700     | 800                  | 900     |
| 37  | 1100            | 900     | 1500                 | 700     |
| 38  | 1200            | 1300    | 1300                 | 1500    |
| 39  | 1700            | 1500    | 1500                 | 1200    |
| 40  | 15,000          | 8000    | 14000                | 9000    |
| 41  | 11000           | 9000    | 10000                | 6000    |

TABLE V

## STATIC RESULTS ACCORDING TO AATC 134-196

| Ex. | Before Cleaning   |         | After Steam Cleaning |         |
|-----|-------------------|---------|----------------------|---------|
|     | Chrome<br>Leather | Neolite | Chrome<br>Leather    | Neolite |
| 42  | 400               | 200     | 500                  | 300     |
| 43  | 600               | 400     | 800                  | 500     |
| 44  | 300               | 600     | 600                  | 700     |
| 45  | 800               | 1100    | 1000                 | 1500    |
| 46  | 500               | 700     | 400                  | 600     |
| 47  | 600               | 500     | 700                  | 700     |
| 48  | 1200              | 1500    | 1500                 | 1900    |
| 49  | 800               | 1100    | 1200                 | 2200    |
| 50  | 400               | 600     | 500                  | 700     |
| 51  | 200               | 400     | 400                  | 600     |
| 52  | 700               | 500     | 800                  | 800     |
| 53  | 1100              | 800     | 1500                 | 1200    |
| 54  | 3200              | 2900    | 4200                 | 3700    |
| 55  | 2800              | 2400    | 3600                 | 4200    |
| 56  | 3700              | 3200    | 3900                 | 3800    |

TABLE V

#### ***<sup>1</sup>Ethoxylated Sorbitol lauric acid ester.***

<sup>2</sup>Humectant was electrolyte.

<sup>3</sup>N-octyl, N-ethyl morpholinium ethosulfate.

<sup>4</sup>Quaternary diethyl sulfate imidazoline.

<sup>5</sup>Untreated control.

TABLE VII

### 'Untreated.'

| Ex. No. | Humectant                   | Parts | Amine Parts     | Wetting Agent Parts | Electrolyte       | Parts | Parts | pH Adjustment Acid | pH      | Textile                       | Percent Coating Weight | Charge Build-up in kv. |
|---------|-----------------------------|-------|-----------------|---------------------|-------------------|-------|-------|--------------------|---------|-------------------------------|------------------------|------------------------|
| 86      | Sorbitol ester <sup>3</sup> | 10    | 10              | 1                   | NaCl              | 1     | 70    | Acetic             | 5.5-6.5 | Taffeta                       | 2                      | 1                      |
| 87      | "                           | 10    | 10              | 1                   | NaCl              | 1     | 70    | "                  | 5.5-6.5 | Taffeta                       | 5                      | 0                      |
| 88      | "                           | 10    | 10              | 1                   | NaCl              | 1     | 70    | "                  | 5.5-6.5 | Taffeta                       | 10                     | 0                      |
| 89      | "                           | 10    | 10              | 1                   | NaCl              | 1     | 70    | "                  | 5.5-6.5 | Nylon rayon filled upholstery | 2                      | 1                      |
| 90      | "                           | 10    | 10              | 1                   | NaCl              | 1     | 70    | "                  | 5.5-6.5 | "                             | 5                      | 5                      |
| 91      | "                           | 10    | 10              | 1                   | NaCl              | 1     | 70    | "                  | 5.5-6.5 | "                             | 10                     | 0                      |
| 92      | Glycerol                    | 20    | 20              | 0                   | CaCl <sub>2</sub> | 5     | 75    | "                  | 6.0-6.5 | Taffeta                       | 2                      | 1                      |
| 93      | "                           | 20    | 20              | 0                   | CaCl <sub>2</sub> | 5     | 75    | "                  | 6.0-6.5 | Taffeta                       | 5                      | 0                      |
| 94      | "                           | 20    | 20              | 0                   | CaCl <sub>2</sub> | 5     | 75    | "                  | 6.0-6.5 | Taffeta                       | 10                     | 0                      |
| 95      | "                           | 20    | 20              | 0                   | CaCl <sub>2</sub> | 5     | 75    | "                  | 6.0-6.5 | Upholstery                    | 2                      | 1                      |
| 96      | "                           | 20    | 20              | 0                   | CaCl <sub>2</sub> | 5     | 75    | "                  | 6.0-6.5 | Upholstery                    | 5                      | 0                      |
| 97      | "                           | 20    | 20              | 0                   | CaCl <sub>2</sub> | 5     | 75    | "                  | 6.0-6.5 | Upholstery                    | 10                     | 0                      |
| 98      | CaCl <sub>2</sub>           | 20    | 20              | 0                   | (5)               | 0     | 100   | "                  | 5.5-6.5 | Taffeta                       | 3                      | 0                      |
| 99      | CaCl <sub>2</sub>           | 20    | 20              | 0                   | (5)               | 0     | 100   | "                  | 5.5-6.5 | Taffeta                       | 5                      | 0                      |
| 100     | CaCl <sub>2</sub>           | 20    | 20              | 0                   | (5)               | 0     | 100   | "                  | 5.5-6.5 | Taffeta                       | 10                     | 0                      |
| 101     | CaCl <sub>2</sub>           | 20    | 20              | 0                   | (5)               | 0     | 100   | "                  | 5.5-6.5 | Upholstery                    | 3                      | 0                      |
| 102     | CaCl <sub>2</sub>           | 20    | 20              | 0                   | (5)               | 0     | 100   | "                  | 5.5-6.5 | Upholstery                    | 5                      | 0                      |
| 103     | CaCl <sub>2</sub>           | 20    | 20              | 0                   | (5)               | 0     | 100   | "                  | 5.5-6.5 | Upholstery                    | 10                     | 0                      |
| 104     | CaCl                        | 30    | 20              | 0                   | (5)               | 0     | 110   | Acetic             | 5.0-5.5 | Taffeta                       | 3                      | 0                      |
| 105     | CaCl <sub>2</sub>           | 30    | 20              | 0                   | (5)               | 0     | 110   | "                  | 5.0-5.5 | Taffeta                       | 5                      | 0                      |
| 106     | CaCl <sub>2</sub>           | 30    | 20              | 0                   | (5)               | 0     | 110   | "                  | 5.0-5.5 | Taffeta                       | 10                     | 0                      |
| 107     | CaCl <sub>2</sub>           | 30    | 20              | 0                   | (5)               | 0     | 110   | "                  | 5.0-5.5 | Upholstery                    | 3                      | 0                      |
| 108     | CaCl <sub>2</sub>           | 30    | 20              | 0                   | (5)               | 0     | 110   | "                  | 5.0-5.5 | Upholstery                    | 5                      | 0                      |
| 109     | CaCl <sub>2</sub>           | 30    | 20              | 0                   | (5)               | 0     | 110   | "                  | 5.0-5.5 | Upholstery                    | 10                     | 0                      |
| 110     | CaCl <sub>2</sub>           | 40    | 20              | 0                   | (5)               | 0     | 120   | "                  | 5.0-5.5 | Taffeta                       | 3                      | 0                      |
| 111     | CaCl <sub>2</sub>           | 40    | 20              | 0                   | (5)               | 0     | 120   | "                  | 5.0-5.5 | Taffeta                       | 5                      | 0                      |
| 112     | CaCl <sub>2</sub>           | 40    | 20              | 0                   | (5)               | 0     | 120   | "                  | 5.0-5.5 | Taffeta                       | 10                     | 0                      |
| 113     | CaCl <sub>2</sub>           | 40    | 20              | 0                   | (5)               | 0     | 120   | "                  | 5.0-5.5 | Upholstery                    | 3                      | 0                      |
| 114     | CaCl <sub>2</sub>           | 40    | 20              | 0                   | (5)               | 0     | 120   | "                  | 5.0-5.5 | Upholstery                    | 5                      | 0                      |
| 115     | CaCl <sub>2</sub>           | 40    | 20              | 0                   | (5)               | 0     | 120   | "                  | 5.0-5.5 | Upholstery                    | 10                     | 0                      |
| 116     | Urea                        | 30    | 10 <sup>1</sup> | 1                   | NaCl              | 1     | 110   | Formic             | 5.0-5.5 | Taffeta                       | 2.5                    | 0-1                    |
| 117     | Urea                        | 30    | 10 <sup>1</sup> | 1                   | NaCl              | 1     | 110   | "                  | 5.0-5.5 | Nylon rayon filled upholstery | 5                      | 0-1                    |
| 118     | Urea                        | 30    | 10 <sup>1</sup> | 1                   | NaCl              | 1     | 110   | "                  | 5.0-5.5 | Nylon rayon non-woven         | 5                      | 5                      |

<sup>1</sup>N-octyl, N-ethyl morpholinium ethyl sulfate.<sup>2</sup>Condensate of tridecyl alcohol with 6 moles of ethylene oxide.<sup>3</sup>Ethoxylated sorbitol lauric acid ester.<sup>4</sup>Nylon-unless otherwise specified.<sup>5</sup>Humectant was electrolyte.

TABLE IX

| Ex. No. | Basic Component | Parts | Organic Acid | Parts | Conductor Parts on Solids Bases | Parts | Electrolyte | Parts (1) | Parts-Water | pH Adjustment | pH  | 02. Per Sq. Yard |
|---------|-----------------|-------|--------------|-------|---------------------------------|-------|-------------|-----------|-------------|---------------|-----|------------------|
| 112     | KOH             | 56    | Formic       | 46    | Naccanol-40 LB.                 | 20    | Na Cl       | 2         | 180         | KOH           | 8.5 | 4                |
| 113     | "               | "     | "            | "     | Nansa HS-55                     | "     | "           | "         | "           | "             | "   | "                |
| 114     | "               | "     | "            | "     | Sodium Lauryl Sulfate           | "     | "           | "         | "           | "             | "   | "                |
| 115     | "               | "     | "            | "     | Alipal CO-433                   | "     | "           | "         | "           | "             | "   | "                |
| 116     | "               | "     | "            | "     | Gaftek 288                      | "     | "           | "         | "           | "             | "   | "                |
| 117     | "               | "     | "            | "     | Nekal BA-75                     | "     | "           | "         | "           | "             | "   | "                |
| 118     | "               | "     | "            | "     | Igepon AP-78                    | "     | "           | "         | "           | "             | "   | "                |
| 119     | "               | "     | "            | "     | Igepon T-33                     | "     | "           | "         | "           | "             | "   | "                |
| 120     | "               | "     | "            | "     | Aerosol OT                      | "     | "           | "         | "           | "             | "   | "                |
| 121     | "               | "     | "            | "     | Triethanol amine Lauryl Sulfate | "     | "           | "         | "           | "             | "   | "                |

TABLE X

Test AATCC -123 -1969  
(all readings in electrostatic volts)

(AFTER STEAM CLEANING)

| Ex. No. | CHROME LEATHER | NEOLITE | CHROME LEATHER | NEOLITE |
|---------|----------------|---------|----------------|---------|
| 112     | +1200          | -900    | +1700          | -1000   |
| 113     | +1500          | -1000   | +1600          | -900    |
| 114     | +1700          | -1200   | +1800          | -1500   |
| 115     | +1100          | -1400   | +1500          | -1200   |
| 116     | +1500          | -900    | +1200          | -1400   |
| 117     | +1900          | -1700   | +2000          | -1900   |
| 118     | +1800          | -2000   | +1700          | -2100   |
| 119     | +1600          | -1800   | +1500          | -2000   |
| 120     | +1100          | -900    | +1200          | -1100   |

55 It is obvious that numerous changes and modifications can be made in the above described details without departing from the spirit and nature of the invention. Therefore, it is to be understood that any such changes and modifications are included within the scope of the invention and that the invention is not to be limited except as set forth in the appended claims.

60 I claim:

1. An antistatic coating composition comprising an aqueous liquid fluid medium having a pH in the range of from about 7 to 13 containing as essential active material a member selected from the group consisting of a. one part by weight of an alkoxylated tertiary amine having the formula



wherein R represents an aliphatic hydrocarbon radical of from about eight to 22 carbon atoms, R' represents a member of the group consisting of hydrogen and methyl and n represents an average integer of from 1 to 51; a quaternary ammonium compound; a phosphate ester; alkali metal salts of C<sub>6-24</sub> sulfated alcohols and sulfonated C<sub>1-6</sub> esters of carboxylic acids; and

b. from 1 to 5 parts by weight of a humectant selected from the group consisting of anionic and nonionic humectants, and when said humectant is a nonionic humectant, a strong electrolyte, said electrolyte being a neutral salt of a strong base and a strong acid.

2. A composition as defined in claim 1, wherein said quaternary ammonium compound is a quaternized copolymer of N-vinyl lactam and a monovinyl monomer copolymerizable therewith.

3. A composition as defined in claim 2, wherein said N-vinyl lactam has the formula



wherein R represents an alkylene bridge group necessary to complete a five, six or seven-membered heterocyclic ring system, R<sub>1</sub> represents hydrogen or a methyl group, and n is at least 3.

4. A composition as defined in claim 1 wherein said quaternary ammonium compound has the formula



wherein R = -(CH<sub>2</sub>)<sub>n</sub>-CH<sub>3</sub> and n = 6 to 26 and R'' and R' = -(CH<sub>2</sub>)<sub>n</sub>-(CH<sub>3</sub> and n = 0 to 6, Y = hydrogen or alkyl.

5. A composition as defined in claim 1 additionally containing .1 to 20% by wt. of a thickening agent.

6. A composition as defined in claim 5, wherein said thickening agent is selected from the group consisting of hydroxyethyl cellulose, methyl cellulose, acrylic acid and starch.

7. A composition as defined in claim 1, said humectant being selected from the group consisting of deliquescent alkali metal salts of lower alkyl carboxylic acids, calcium carbonate, glycerol, urea, ethylene glycol, sorbitol, ethoxylated sorbitol lauric acid esters, and mixtures thereof.

8. A composition as defined in claim 1, wherein the humectant is calcium chloride.

9. A composition as defined in claim 1, wherein the humectant is a deliquescent alkali metal salt of a lower alkyl carboxylic acid having from one to four carbon atoms and there is present as an electrolyte at least 0.01 parts by weight of a compound selected from the group consisting of sodium chloride and calcium chloride.

10. A composition as defined in claim 1, wherein the humectant is a nonionic humectant selected from the group consisting of sorbitol humectants, glycerol and urea, and there is present as an electrolyte at least 0.01 parts by weight of an electrolyte selected from the group consisting of sodium chloride and calcium chloride.

11. A composition as defined in claim 1, wherein said humectant is an ethoxylated sorbitol lauric acid ester.

12. A composition as defined in claim 1, wherein component (a) is N-octyl-N-ethyl morpholinium ethosulfate.

13. A composition as defined in claim 1, wherein component (a) is a phosphate ester.

14. A composition as defined in claim 13, wherein said phosphate ester is a phosphate ester of a nonionic surface active condensation product of at least 1 mole of ethylene oxide with 1 mole of a compound containing at least six carbon atoms and a reactive hydrogen atom.

15. A process for the preparation of an antistatic coating composition comprising an aqueous liquid fluid medium having a pH in the range of from about 7 to 13 and containing as essential active material a member selected from the group consisting of

a. one part by weight of an alkoxylated tertiary amine having the formula



wherein R represents an aliphatic hydrocarbon radical of from about eight to 22 carbon atoms, R' represents a member of the group consisting of hydrogen and methyl and n represents an average integer of from 1 to 51; a quaternary ammonium compound; a phosphate ester; alkali metal salts of C<sub>6-24</sub> sulfated alcohols and sulfonated C<sub>1-6</sub> esters of carboxylic acids; and

b. from 1 to 5 parts by weight of a humectant selected from the group consisting of anionic and nonionic humectants, and when said humectant is a nonionic humectant, a strong electrolyte, said electrolyte being a neutral salt of a strong base and a strong acid, comprising adding substantially equimolar amounts of an alkali metal base and an aliphatic carboxylic acid having from one to four carbon atoms to water to thereby produce the humectant in situ, adding thereto the active material and thoroughly mixing the same to obtain a uniform composition, and adding to the mixture a neutralizing base in such amount as to adjust the pH of such mixture within the range of 7-13.

16. The process of claim 15, further comprising thickening said composition with a thickening agent selected from the group consisting of hydroxyethyl cellulose, methyl cellulose, acrylic acid and starch.

\* \* \* \* \*